

# UNITED STATES PATENT OFFICE.

HERBERT P. PEARSON, OF NEW YORK, N. Y., ASSIGNOR TO PEARSON PRODUCTS CORPORATION, OF NEW YORK, N. Y., A CORPORATION OF NEW YORK.

## METHOD OF WATERPROOFING FABRICS.

1,307,373.

Specification of Letters Patent. Patented June 24, 1919.

No Drawing.

Application filed April 3, 1919. Serial No. 287,194.

To all whom it may concern:

Be it known that I, HERBERT P. PEARSON, a subject of the United Kingdom of Great Britain, residing at two hundred West Seventy-eighth street, in the county of New York and State of New York, have invented certain new and useful Improvements in Methods of Waterproofing Fabrics, of which the following is a specification.

10 This invention relates to the water-proof finishing of textile fabrics and wearing apparel, including such a variety as felt hats and ostrich feathers, and more especially to the production of improved transparent, 15 semi-transparent or invisible water-proof coatings on the fibers of the same through the agency of a compound of semi-solid and solid hydro-carbons in conjunction with siccative oils treated with selenium salts. 20 Heretofore it has been customary in this field to make use of the solid residues of petroleum, basic salts of fatty acids and insoluble mineral salts, to all of which objection has been raised that they either stiffen 25 the fiber or give the fabric a harsh handle when used in sufficient quantities to produce the desired resistance to water, and moreover that they are subject to physical or chemical changes during those finishing 30 operations employing great heat which are applied to textile fabrics and wearing apparel.

It has been regarded as desirable in the water-proof finishing of textile fabrics and 35 wearing apparel to secure prevention of the stiffening of the fabric while producing the maximum resistance to wetting by water. To this end I make use in the present invention of compounds composed of solid 40 hydro-carbons and petroleum residues preferably paraffin waxes of melting point below 135 degrees Fahrenheit, in conjunction with a petrolatum free from mineral oils of light gravity and in conjunction with a siccative 45 oil preferably Chinese wood oil or Perrilla oil treated with a selenium salt or with selenium oxid.

The addition of vegetable drying oils

alone to textile fabrics has resulted in the slow oxidation of the oils with the formation of linoxyns, which end products I regard as undesirable because of the stiffening of the fiber resulting after drying. By the addition of selenium compounds to the siccative oils I have destroyed the tendency of the oils to dry and caused them to form a soft, elastic, slowly oxidizable complex, that in conjunction with solid viscous or semi-solid petroleum residues produces a mass soluble in petroleum distillates which has valuable water-proofing properties in the treatment of textile fabrics and wearing apparel. I am unable to state whether the combinations taking place between the selenium treated siccative oils and the petroleum residues are actual chemical compounds or whether the occlusive action of the selenium tungates (in the case of Chinese wood oil) is responsible for the composition of the resulting body. The action may be chemical or adsorptive.

The compositions embodied under my invention are therefore those which comprise paraffins and petrolatums intimately associated with selenium tungate in lesser proportion. I realize that the composition may be greatly varied and still satisfy the specific conditions mentioned above and all such variation I regard as within the scope of my invention.

A formula indicative of the present invention is as follows:

80 lbs. of paraffin wax of 122 degrees Fahrenheit melting point, and 20 lbs. of petrolatum, thoroughly mixed and combined under heat with 8 lbs. of Chinese wood oil previously treated with 1% of selenium oxid. The process of treating the Chinese wood oil is as follows: The oil is heated to a temperature of 400 degrees Fahrenheit when the selenium oxid is added and for two hours the oil is slowly raised with stirring to a temperature not exceeding 550 degrees Fahrenheit, the entire mass being then allowed to cool to room temperature.

95 My compositions may be applied with a

brush or dissolved in a suitable solvent and the fabric impregnated therewith or applied with a spray or by means of spreading rollers.

5 I claim:

1. The process of water-proof finishing textile fabrics and wearing apparel which comprises their treatment with paraffin wax

in conjunction with petrolatum and a selenium treated Chinese wood oil.

2. The process of water-proof finishing textile fabrics and wearing apparel which comprises their treatment with solutions in volatile solvents of paraffin wax, petrolatum and selenium treated Chinese wood oil.

HERBERT P. PEARSON.